

# United States Patent Office.

EVANDER W. RANNEY, OF NEW YORK, N. Y.

Letters Patent No. 98,522, dated January 4, 1870.

## IMPROVED COMPOSITION FOR CONCRETE PAVEMENTS.

The Schedule referred to in these Letters Patent and making part of the same.

*To all whom it may concern:*

Be it known that I, EVANDER W. RANNEY, of New York, county and State of New York, have invented a new and improved Asphaltic Pavement; and I do hereby declare that the following is a full and exact description thereof.

The nature of my invention consists in a composition of broken stone or gravel, native or artificial asphaltum, and pine or coal-tar, mixed in such proportions as to form a pasty substance, which, when spread on a suitable foundation, and thoroughly rolled or pressed together, makes a durable yet elastic pavement for road-beds, walks, floors, roofs, and similar purposes.

To enable those skilled in the art to make and use my invention, I will proceed to describe its composition, and the manner of making and using the same.

I take, gravel or broken stone, six bushels; asphaltum, either native or artificial, ten quarts; pine or coal-tar, eighteen quarts; and add, to every five hundred pounds of said composition, one pound of bichromate of potash.

The asphaltum and tar are put into separate kettles and heated till they are at their greatest fluidity, which will be about the temperature of boiling water, and then they are mixed together in the above proportions, when the native asphalt is used; but if it be the artificial asphalt, I mix them in equal parts.

The gravel or broken stone is made perfectly dry, and heated till it is about the same temperature of the asphalt-mixture.

I then put in a pile six bushels of the hot gravel and add to it twenty-eight quarts of the asphalt-mixture, and I thoroughly mix the compound, either by hand or by machinery, till every particle of the gravel is well smeared with the liquid.

I then take the mixture to the bed previously prepared for it, and spread evenly over the surface while yet warm, and thoroughly roll the same with heavy rollers till the whole mass is thoroughly compacted together.

The bed or foundation may be the ordinary soil, or gravel, made hard and smooth with heavy rollers; or it may be of stone, wood, or brick.

For a road-bed or street-pavement, with a sand or gravel foundation, the concrete should be five or six inches thick when finished, and be laid in not less than two layers or coats. The first layer may be of such material as would pass through a screen with a three-inch mesh, and laid four inches thick, while the material for the second coat should pass through a screen with a one-and-a-half-inch mesh, and be finished about two inches thick.

When the concrete is laid on stone pavement, the gravel should pass through a screen with a mesh of

one and a half inch, and be laid with one or two coats, about three inches in thickness.

Fine sand or any fine hard substance, as iron-ore or mineral paint, may be sprinkled over the concrete immediately before or after the first rolling, which will give it a smooth, compact surface.

The quantity of the tar and asphalt-mixture will vary somewhat with the degree of fineness of the gravel.

If very coarse, and little fine mixed with it, twenty quarts of the mixture will suffice for six bushels of the gravel; or, if it is very fine, with a large proportion of sand, it will require as much as thirty to thirty-four quarts to the six bushels of gravel.

The proportions of tar and asphalt will also vary somewhat with the season of the year.

One object of the asphalt is to harden the composition, and in very warm weather equal parts of native asphalt and tar, or two parts of artificial asphalt to one part of tar, may be used; while in very cold weather about one part of the native asphalt and two parts of the artificial asphalt may be used, with three and even four parts of tar.

I prefer the ordinary pine-tar of commerce for my use, though coal-tar makes very good work, when mixed with the asphalt as above. And I have sometimes mixed the two tars in about equal parts with very good effect.

When hard and durable rock can be obtained, and thoroughly crushed, and mixed with the gravel in about equal parts, I prefer it to either one entirely.

When gravel or broken stone cannot be obtained, I use sea-shells, iron-ore, or iron-slag, or any rough, hard, durable substance, reduced to a proper fineness, as a substitute for gravel.

When the weather is quite cold, it will facilitate the thorough packing of the concrete by using hot rollers.

Walks, foot-paths, and floors can be walked over as soon as finished. Carriage-roads and street-pavements may be used generally within twenty-four hours; but sometimes three to five days will be required to get thoroughly hardened.

What I claim as my invention, and desire to secure by Letters Patent of the United States, is—

A concrete pavement, composed of the materials and prepared and laid substantially in the manner herein described.

In testimony whereof I have signed my name to this specification in the presence of two subscribing witnesses.

EVANDER W. RANNEY.

Witnesses:

FRANK S. HOLMES,  
JAMES GREEN.